

## UNITED STATES PATENT OFFICE

FRANK C. MATHERS, OF BLOOMINGTON, INDIANA, AND LOUIS BATEMAN, OF EAST LANSING, MICHIGAN, ASSIGNEES TO UNITED STATES SMELTING, REFINING & MINING COMPANY, OF PORTLAND, MAINE, A CORPORATION OF MAINE

## ELECTRODEPOSITION OF METALS

No Drawing.

Application filed January 9, 1931. Serial No. 507,754.

The invention relates to electrodeposition of metals and more particularly to electrolytic refining of lead by electrodeposition of the metal from aqueous solutions of its salts. 5 It is the practice in the electrolytic refining of metals to employ so-called addition reagents in aqueous solutions of the compounds of the metals from which the metals are deposited. The rôle which such addition 10 reagents plays in the actual electrodeposition of metals is not understood, but their use results in the production of smooth deposits which are so finely crystalline that they may be considered as being substantially non-crystalline. 15 The present invention is based on the discovery of new reagents of this character for use with an electrolyte containing dithionic acid in the electrodeposition of lead, which process has marked advantages over 20 prior reagents employed. The proper amount of reagent to be used depends upon the chemical composition, the temperature, and the rate of circulation of the electrolyte, the amount and character of the impurities in the 25 electrolyte, and the current density employed.

The new reagents are classified as hydroxy compounds of coal tar which include phenol, resorcinol, cresol, and beta-naphthol. Cresol is an example of this class of hydroxy compounds of coal tar which may be used as addition reagents with especially good results, but it will be understood that, except as limited by the terms of the claims, the invention also includes the use of the others in the above 35 category.

We have discovered in the electrolytic refining of lead that hydroxy compounds of coal tar, such, for instance, as cresol, may be used as an addition reagent in dithionic acid 40 electrolytes with remarkable advantageous results. It may be used to replace many of the addition reagents now commonly used and because of its comparatively low cost, substantial economy may be thereby effected. 45 It may be used alone or in partial replacement of some of the commonly used addition reagents, effecting not only an economy thereby, but permitting a substitution to take place in old electrolyte, thus avoiding the cost of 50 new electrolyte when changing over to this

new addition reagent. In many cases, it produces a deposit of the lead upon the cathode superior to deposits obtained by other addition reagents, increasing thereby the efficiency of the operation, and resulting in important economy in the power consumption. No accumulation in the electrolyte of substances which might finally cause the formation of non-adherent and coarsely crystalline deposits has been noticed when this addition reagent is used, as has been noticed when certain addition reagents heretofore known have been used.

While cresol alone or in combination with other addition reagents gives satisfactory results with a dithionic acid electrolyte, a mixture of cresol and glue is preferred, especially as the combination is more economical than the use of cresol alone. Other substances belonging to the coal tar hydroxy compounds 60 may similarly be used as for instance, instead of using cresol with glue, resorcinol or beta-naphthol give excellent results. Likewise phenol (carbolic acid) and glue and pyrogallol and glue give satisfactory results 65 in the dithionic acid electrolyte.

The composition of the electrolyte may vary and likewise the amounts of reagents may vary without materially affecting the character of the deposit. An electrolyte containing 5% lead dithionite and 2% free dithionic acid to which has been added .8% cresol and .15% glue has given a satisfactory cathode deposit and a high current efficiency. With the same electrolyte good 70 deposits have been obtained with .04% beta-naphthol and .02% glue and likewise with 1% phenol and .25% glue.

Having thus described the invention, what 75 is claimed is:

1. That improvement in the electrodeposition of lead from electrolytes containing dithionic acid which consists of the use of a hydroxy compound occurring in coal tar as 80 an addition reagent in the acid electrolyte.
2. That improvement in the electrodeposition of lead from electrolytes containing dithionic acid which consists of the use of a cyclic hydroxy compound occurring in coal 85

tar as an addition reagent in the acid electrolyte.

3. That improvement in the electrodeposition of lead from electrolytes containing dithionic acid which consists of the use of a compound of a class consisting of phenol, cresol, resorcinol and beta-naphthol as an addition reagent in conjunction with glue in the acid electrolyte.
- 10 4. That improvement in the electrodeposition of lead from electrolytes containing dithionic acid which consists of the use of a hydroxy compound occurring in coal tar in conjunction with glue as an addition reagent in the acid electrolyte.
- 15 5. That improvement in the electrodeposition of lead from electrolytes containing dithionic acid which consists of the use of a cyclic hydroxy compound occurring in coal
- 20 tar in conjunction with glue as an addition reagent in the acid electrolyte.
- 25 6. That improvement in the electrodeposition of lead from electrolytes containing dithionic acid which consists of the use of a compound of a class consisting of phenol, cresol, resorcinol, and beta-naphthol as an addition reagent in conjunction with other addition reagents in the acid electrolyte.
- 30 7. That improvement in the electrodeposition of lead from electrolytes containing dithionic acid which consists in the use of a compound of the class consisting of phenol, cresol, resorcinol, and beta-naphthol as an addition reagent.
- 35 In testimony whereof we have signed our names to this specification.

FRANK C. MATHERS.  
LOUIS BATEMAN.

40

45

50

55

60

65